

## UNITED STATES PATENT OFFICE

2,289,805

## SULPHONIC ESTER COUPLER

Henry Dudley Porter and Arnold Weissberger,  
Rochester, N. Y., assignor to Eastman Kodak  
Company, Rochester, N. Y., a corporation of  
New Jersey

No Drawing. Application September 26, 1940, Se-  
rial No. 358,493. In Great Britain January 3,  
1940

15 Claims. (CL 95—6)

This invention relates to color-forming de-  
velopment and particularly to novel coupling  
components for producing colored images.

It is known that colored photographic images  
may be formed by using a developer which forms  
a colored compound on development. The  
colored compound thus formed is deposited ad-  
jacent to the silver grains of the silver image  
during the development. It is also known that  
a colored image may be formed by adding to  
certain developer solutions or by incorporating in  
the gelatino-silver-halide emulsion before or  
after exposure a compound which couples during  
development with the oxidation product of  
the developing agent and forms a coloring sub-  
stance which is likewise deposited adjacent to  
the silver grains of the silver image during de-  
velopment. Such a compound, which is em-  
ployed in conjunction with a developing agent  
for the silver and which couples with the oxida-  
tion product thereof during development, is re-  
ferred to herein as a coupling component or  
coupler.

The present invention concerns new or im-  
proved color forming developers comprising a 25  
primary aromatic amino compound, serving as  
the developing agent, and a coupler as herein-  
after defined and also includes a new or improved  
color development process which consists in de-  
veloping a reducible silver salt image in a photo-  
graphic element with the aid of a primary aromatic  
amino compound in the presence of a  
coupler as hereinafter defined. It also includes  
photographic sensitive elements having such a  
coupler incorporated in one or more emulsion  
layers.

In British Patent 503,752 sulphonic ester cou-  
plers are described which are obtained by the  
reaction of  $\alpha$ -naphthol sulphonic acid chloride  
with phenols having a high molecular substituted  
amino or hydroxy group. In these couplers the  
hydroxyl group of the naphthol constitutes the

alcohol or an alkoxy or aryloxy alcohol, or with  
a phenol. According to the molecular size and  
solubility of these compounds, they may be in-  
corporated either in photographic emulsions or  
in developing solutions. The introduction of the  
sulphonic ester group tends to confer better dis-  
persability on the coupler molecule, which is a  
desirable property when the coupler is to be in-  
corporated in emulsions.

The compounds which we propose to use have  
the following general formula:



wherein

R=an aroyl acetaminobenzene

Y=alkyl, aryl, alkoxy alkyl, or aryloxy alkyl

Specific compounds which may be used ac-  
cording to our invention are the following:

(1)



Methyl p-(benzoylacetamino) benzenesulphonate

(2)



Ethyl p-(benzoylacetamino) benzenesulphonate

(3)



n-Propyl p-(benzoylacetamino) benzenesulphonate

(4)



<math>\beta</math>-Ethoxyethyl p-(benzoylacetamino) benzenesulphonate

(5)



<math>\beta</math>-Benzoyloxyethyl p-(benzoylacetamino) benzenesulphonate

(6)



Ethylene <math>\alpha,\beta</math> di-(p-benzoylacetamino) benzenesulphonate

(7)



n-Amyl p-(benzoylacetamino) benzenesulphonate

"coupling function" and the couplers, therefore,  
produce blue or blue-green dyes on development  
in the presence of suitable developing agents.  
They are, moreover, suitable for use only in 50  
emulsion layers.

We have found that sulphonic ester couplers  
capable of producing yellow dyes may be pre-  
pared by treating a sulphonic acid chloride of  
a yellow coupler with an alcohol, such as ethyl 55

(8)

 $\beta$ -( $\beta$ -n-Butoxyethoxy) ethyl p(benzoylacetamino) benzene-sulphonate

(9)

 $\beta$ -( $\beta$ -Benzoyloxyethoxy)-ethyl p(benzoylacetamino) benzenesulphonate

(10)

 $\beta$ -( $t$ -Butylphenoxy) ethyl p(benzoylacetamino) benzenesulphonate

(11)



2,4-diamylphenyl p(benzoylacetamino)-benzenesulphonate

(12)

 $\beta$ -( $t$ -Butylphenoxy-ethyl p-anisoylacetamino-benzenesulphonate

(13)



n-Amyl p-anisoylacetamino-benzenesulphonate

The couplers made according to our invention may be dissolved in the developing solution or may be incorporated in the emulsion layer according to their solubility characteristics. Compounds 1 to 4 are suitable for use in the developing solution and compounds 5 to 13 may be incorporated in the emulsion layer.

As stated above, the coupler must contain a coupling function, which in this case is a reactive methylene group. By "coupling function" we mean a functional or reactive group common to coupler compounds which react with primary aromatic amino developing agents. By "reactive methylene" we mean a  $\text{CH}_2$  group which is reactive in the coupling process. The  $\text{CH}_2$  group is usually present between two negative centers as in the groups  $-\text{CO}-\text{CH}_2-\text{CO}$  or  $-\text{CO}-\text{CH}_2-\text{CN}$ , in the case of the present compounds, the former. One of the hydrogen atoms of the methylene group may, in general, be substituted without destroying the chemical activity of the group.

The coupling compounds used according to our invention may contain other substituents which do not affect the coupling properties of the compound. Where we refer in the general formula

to alkoxy and aryloxy groups, it is to be understood that these groups may be further substituted provided that the other requirements with respect to coupling are met.

5 The aromatic amino developing agents used with the coupler compounds of our invention include the mono-, di and tri-aminoaryl compounds and their derivatives formed by substitution in the amino group as well as in the ring, 10 such as alkylphenylenediamines and alkyltoluyl-enediamines. These compounds are usually used in the salt form, such as the hydrochloride or the sulphate, which are more stable than the amines themselves. Suitable compounds are di- 15 ethyl-p-phenylenediamine hydrochloride, mono-methyl-p-phenylenediaminehydrochloride, di-methyl-p-phenylenediaminehydrochloride and dimethyl-p-phenylenediamine sulphate. The p-aminophenols and their substitution products may also be used where the amino group is un- 20 substituted. All of these compounds have an unsubstituted amino group which enables the oxidation products of the developer to couple with the color forming compounds to form a dye image.

25 The following developer formula may be used with the compounds of our invention:

A. p-Aminodiethylaniline sulphate grams 2  
Sodium sulphite anhydrous do 5  
30 Sodium carbonate anhydrous do 20  
Potassium bromide do 2  
Water to liter 1  
B. Coupler grams 1 to 5  
35 Isopropyl alcohol cc 100

B is added to A

Our development process may be employed for the production of colored photographic images 40 in layers of gelatin or other carrier such as collodion, organic esters of cellulose or synthetic resins. The carrier may be supported by a trans-

parent medium such as glass, a cellulose ester, or a non-transparent reflecting medium such as paper or an opaque cellulose ester. The emulsion 50 may be coated as a single layer on the support or as superposed layers on one or both sides of the support. The superposed layers may be differentially sensitized to form natural color photographic images in the well known manner.

55 The couplers which we propose to use are prepared, in general, by the interaction of the sulphonyl chloride of the coupler with the appropriate alcohol in the presence of one equivalent of pyridine. For example, to prepare methyl-p-(benzoylacetamino)-benzenesulphonate, one equivalent weight of p-(benzoylacetamino)-benzene-sulphonyl chloride is reacted with an excess methyl alcohol in the presence of one equivalent weight of pyridine. In the case of 60 the couplers prepared from the sulphonyl chloride of the coupler and a phenol, the sulphonyl chloride is reacted with the sodium salt of the phenol in xylene solution. For example, Compound 11, 2,4-diamylphenyl-p-(benzoylacetamino)-benzenesulphonate, the coupler was obtained by the reaction of p-(benzoylacetamino)-benzene sulphonyl chloride on the sodium salt of 65 2,4-diamylphenol in xylene solution.

70 The sulphonyl chlorides of the couplers are prepared as described in our copending applica- 75

tion Serial No. 358,494, filed September 26, 1940, by treating the appropriate acetanilide with chlorosulphonic acid at a temperature below about 10° C. and permitting the reaction to proceed for a short time, that is, of the order of a few days. For example, p-benzoylacetaminobenzenesulphonyl chloride is prepared as follows:

**EXAMPLE.—p-Benzoylacetaminobenzene-sulphonyl chloride**

One part of benzoylacetanilide is added to 2 volumes of chlorosulphonic acid while keeping the temperature below 10° C. The reaction mixture is allowed to warm slowly to room temperature, and, after standing overnight, is decomposed by pouring onto ice. The product is filtered, washed with water, dried in ether solution, and recrystallized from benzene. M. P. 149-151° C.

The example and compounds set forth in the present specification are illustrative only and it is to be understood that our invention is limited only by the scope of the appended claims.

We claim:

1. A color forming photographic developer comprising a primary aromatic amino developing agent and a coupler compound having the formula:



where R is an aroyl acetaminobenzene and Y is selected from the group consisting of alkyl, aryl, alkoxyalkyl and aryloxyalkyl radicals.

2. A color forming photographic developer comprising a primary aromatic amino developing agent and a coupler compound having the formula:



where R is a p-benzoylacetaminobenzene and Y is selected from the group consisting of alkyl, aryl, alkoxyalkyl and aryloxyalkyl radicals.

3. A color forming photographic developer comprising a primary aromatic amino developing agent and a coupler compound having the formula:



where R is a p-benzoylacetaminobenzene and Y is an alkyl radical.

4. A color forming photographic developer comprising a primary aromatic amino developing agent and a coupler compound having the formula:



where R is a p-benzoylacetaminobenzene and Y is an alkoxyethyl radical.

5. A color forming photographic developer comprising a primary aromatic amino developing agent and a coupler compound having the formula:



where Y is selected from the group consisting of alkyl, aryl, alkoxyalkyl, and aryloxyalkyl radicals.

6. The method of producing a colored photographic image in a gelatino silver halide emulsion layer which comprises exposing the layer and developing it with a primary aromatic amino developing agent in the presence of a coupler compound having the formula:



where R is an aroyl acetaminobenzene and Y 75

is selected from the group consisting of alkyl, aryl, alkoxyalkyl and aryloxyalkyl radicals.

7. The method of producing a colored photographic image in a gelatino silver halide emulsion layer which comprises exposing the layer and developing it with a primary aromatic amino developing agent in the presence of a coupler compound having the formula:



where R is a p-benzoylacetaminobenzene and Y is selected from the group consisting of alkyl, aryl, alkoxyalkyl and aryloxyalkyl radicals.

8. The method of producing a colored photographic image in a gelatino silver halide emulsion layer which comprises exposing the layer and developing it with a primary aromatic amino developing agent in the presence of a coupler compound having the formula:



where R is a p-benzoylacetaminobenzene and Y is an alkyl radical.

9. The method of producing a colored photographic image in a gelatino silver halide emulsion layer which comprises exposing the layer and developing it with a primary aromatic amino developing agent in the presence of a coupler compound having the formula:



where R is a p-benzoylacetaminobenzene and Y is an alkoxyethyl radical.

10. The method of producing a colored photographic image in a gelatino silver halide emulsion layer which comprises exposing the layer and developing it with a primary aromatic amino developing agent in the presence of a coupler compound having the formula:



where Y is selected from the group consisting of alkyl, aryl, alkoxyalkyl, and aryloxyalkyl radicals.

11. A photographic emulsion for forming colored images comprising a carrier containing a sensitive silver halide and a coupler compound having the formula:



where R is an aroyl acetaminobenzene and Y is selected from the group consisting of alkyl, aryl, alkoxyalkyl and aryloxyalkyl radicals.

12. A photographic emulsion for forming colored images comprising a gelatino silver halide emulsion having incorporated therein a coupler compound of the general formula:



60 where R is a p-benzoylacetaminobenzene and Y is selected from the group consisting of alkyl, aryl, alkoxyalkyl and aryloxyalkyl radicals.

13. A photographic emulsion for forming colored images comprising a gelatino silver halide emulsion having incorporated therein a coupler compound of the general formula:



where R is a p-benzoylacetaminobenzene and Y is an alkyl radical.

14. A photographic emulsion for forming colored images comprising a gelatino silver halide emulsion having incorporated therein a coupler compound of the general formula:



where R is a p-benzoylacetaminobenzene and Y is an alkoxyethyl radical.

15. A photographic emulsion for forming colored images comprising a gelatino silver halide emulsion having incorporated therein a coupler compound of the general formula:



where Y is selected from the group consisting of alkyl, aryl, alkoxyalkyl, and aryloxyalkyl radicals.

HENRY DUDLEY PORTER.  
ARNOLD WEISSBERGER.